

## [54] SILVER HALIDE PHOTOGRAPHIC LIGHT-SENSITIVE MATERIAL AND IMAGE FORMING METHOD

[75] Inventors: Tsumoru Ishii; Shinji Sakaguchi, both of Minami-ashigara, Japan

[73] Assignee: Fuji Photo Film Co., Ltd., Kanagawa, Japan

[21] Appl. No.: 279,401

[22] Filed: Jul. 1, 1981

## [30] Foreign Application Priority Data

Jul. 1, 1980 [JP] Japan ..... 55-89863

[51] Int. Cl.<sup>3</sup> ..... G03C 5/26

[52] U.S. Cl. ..... 430/403, 430/434; 430/523; 430/536; 430/950; 430/961

[58] Field of Search ..... 430/950, 961, 523, 536, 430/537, 434, 403

## [56] References Cited

## U.S. PATENT DOCUMENTS

|           |        |                  |         |
|-----------|--------|------------------|---------|
| 3,079,257 | 2/1963 | Morcher et al.   | 430/950 |
| 3,370,951 | 2/1968 | Hasenauer et al. | 430/950 |
| 3,632,342 | 1/1972 | Salesin et al.   | 430/950 |
| 4,022,622 | 5/1977 | Timmerman et al. | 430/950 |
| 4,094,848 | 1/1978 | Naito            | 430/950 |
| 4,142,894 | 3/1979 | Hori et al.      | 430/950 |

Primary Examiner—Mary F. Downey  
 Attorney, Agent, or Firm—Sughrue, Mion, Zinn,  
 Macpeak and Seas

## [57] ABSTRACT

A silver halide photographic light-sensitive material is

described containing in its outermost layer a high molecular weight matting agent formed from at least one kind of alkali insoluble synthetic polymer grains having a glass transition point of at least 60° C. and an average grain size of from 0.2 to 10, and said polymer is represented by the formula (I):



wherein A represents a divalent group derived from at least one monomer having the formula (II); B represents a divalent group derived from at least one monomer having the formula (III), whose homopolymer has a glass transition point of at least 50° C.; C represents a divalent group derived from an ethylenic unsaturated monomer other than A or B which is capable of copolymerizing with the monomers forming both A and B; x represents the fractional content of group A, which ranges from 0.005 to 0.20 mol/mol of polymer of formula (I); y represents the fractional content of group B, which ranges from 0.50 to 0.995 mol/mol of polymer of formula (I); and z represents the fractional content of group C, which ranges from 0 to 0.495 mol/mol of polymer of formula (I). Formula (II) and formula (III) are disclosed herein.

These polymer grains are not removed from the outermost layer by rapid development-processing and exhibit a satisfactory matting effect even after the completion of such processing.

21 Claims, No Drawings

**SILVER HALIDE PHOTOGRAPHIC  
LIGHT-SENSITIVE MATERIAL AND IMAGE  
FORMING METHOD**

**FIELD OF THE INVENTION**

This invention relates to a silver halide photographic light-sensitive material and, more particularly, to an image-forming method in which a silver halide photographic light-sensitive material (referred to simply as the "sensitive material" hereinafter) containing a high molecular weight matting agent in its outermost layer is employed.

**BACKGROUND OF THE INVENTION**

In general, a sensitive material has an outermost layer (surface layer) which contains as a binder a certain hydrophilic organic colloid whose representative is gelatin. Therefore, the sensitive material shows an increase in its adhesiveness or tackiness under circumstances of high temperature and humidity, whereby adhesion occurs readily when the sensitive material is allowed to stand in contact with another object.

This adhesion phenomenon occurs between sensitive materials, or between a sensitive material and a different material placed in contact therewith upon production of the sensitive material or during storage, photographing, processing or projection, or during preservation of the processed sensitive material, and it often causes serious disadvantages.

It is well-known in this art that in order to solve this problem an inorganic substance such as silicon dioxide, magnesium oxide, titanium dioxide, calcium carbonate or the like, or fine grains of an organic substance such as polymethyl methacrylate, cellulose acetate propionate or the like (which are called "matting agent" hereinafter) is incorporated in the topmost layer of a sensitive material and thereby the surface of the sensitive material is increased in its roughness, that is to say, it is matted and reduces its adhesiveness.

In some cases it is desired to remove a matting agent for the purposes of improving transparency and graininess properties of formed images. Such a method is described in U.S. Pat. No. 4,142,894, which describes methyl methacrylate-methacrylic acid copolymers intended to be soluble in an alkaline processing solution at a temperature above 30° C. On the other hand, in other photographic materials it is desired to retain the matting agent to prevent the adhesion phenomenon after developing, and to prevent removal of matting agent and related problems during image development processing.

On the other hand, recent development-processing techniques for sensitive materials have been increasingly rapid. In proportion, as the processing time becomes shorter, the sensitive material carries a larger amount of processing solution used in the previous processing step into the processing bath subsequent thereto and, consequently, the processability of the processing bath deteriorates more rapidly. In addition, an increased water content in the final processing bath imposes heavier load on the drying system, and, consequently, makes a rapid processing more difficult.

Under these circumstances, various devices have been tried with the intention of reducing the quantity of a processing solution which is carried out of the processing bath used in one step into another processing bath to be used in the following step.

For instance, in the case that a number of narrow belt-form films, such as color sensitive materials having a width of 35 mm, are linked up one after another, and subjected continuously to a chain of processings, a rubber plate for removing excess liquid (which is referred to as a "rubber lip" hereinafter) has been set up between each pair of processing baths arranged in order and/or behind the last processing bath, and the sensitive materials are drawn through the rubber lips and thereby the processing solutions adhering to the sensitive material are scraped off respectively. In another case that sheet-form sensitive materials, such as X-ray sensitive materials, are processed, a pair of counter rollers is set up between every pair of processing baths arranged in order and/or behind the last processing bath, and the sensitive materials are drawn through pairs of rollers and thereby the processing solutions adhering to the sensitive material are squeezed respectively. Rollers used for this purpose are called "squeeze rollers". Furthermore, "buff rollers" can be also used to remove excess processing solutions from the sensitive materials.

Thus, as a chain of processings of sensitive materials is carried out at higher speed, the extent of damage from abrasion which is caused in the surface of a sensitive material by the sensitive material being passed through the rubber lips, the squeeze rollers or the buff rollers becomes more drastic.

When the surface of a sensitive material is rubbed severely with rubber lips, squeeze rollers or buff rollers, problems such that matting agent present in the outermost layer is removed from the layer are apt to be caused.

Removal of the matting agent due to passage through rubber lips or squeeze rollers results in a low degree of matting for the sensitive material after the completion of a chain of processings, and tends to cause adhesion between sensitive materials or between the sensitive material and other materials and thereby causing various problems. Furthermore, upon contact exposure of another unexposed sensitive material through the sensitive material having received processings in the above-described manner there is a possibility of generation of the so-called "Newton ring" due to a low degree of matting (the extent of matting is expressed in the term of "mat property" hereinafter).

More importantly, removed particles of the matting agent are accumulated, aggregate, grow into huge grains, and some of resulting huge grains of the matting agent are transferred onto the surfaces of other sensitive materials.

Adhesion of such huge grains to the surfaces of sensitive materials makes the sensitive materials dirty and causes severe damage to the quality of the sensitive materials finished processings.

Furthermore, the huge grains of a matting agent accumulated on the surface of a rubber lip or a squeeze roller impair the surface of a sensitive material conveyed with a high speed, and in some cases may make scratches on the surface of the sensitive material.

A scratch having once been generated, a lot of defective materials are produced for a short time because of high processing and conveying speeds, to result in a heavy loss.

In addition, although fine grains of silicon dioxide have generally been employed as a matting agent in this art, such a matting agent suffer from the defect that it is impossible to control their average grain size to the degree desired.

Moreover, fine grains of silicon dioxide are likely to adhere to wall surfaces of a dissolution tank and so on in the step of preparing a coating solution for making a hydrophilic colloidal layer of a sensitive material, for example, a surface protecting layer and, therefore, they suffer from a troublesome disadvantage that the cleaning work in the preparation step requires extensive labor.

### SUMMARY OF THE INVENTION

Therefore, an object of this invention is to provide a sensitive material which exhibits a satisfactory mat property even after the completion of development-processing without causing removal of a matting agent in the processing step, even in the rapid development-processing step.

Another object of this invention is to provide a sensitive material in which a matting agent is used whose grain size may be easily controlled, and whose grains do not firmly stick on wall surfaces of a dissolution tank and the like in the step of producing the sensitive material.

The above-described objects of this invention are attained with a sensitive material which has on a support at least one light-sensitive silver halide emulsion layer, said material containing in its outermost layer at least one kind of alkali insoluble synthetic polymer grains having a glass transition point of at least 60° C. and an average grain size of 0.2 $\mu$  to 10 $\mu$ , and said polymer is represented by formula (I):



wherein A represents a divalent group derived from at least one monomer having the formula (II) (illustrated below); B represents a divalent group derived from at least one monomer having the formula (III) (illustrated below) whose homopolymer has a glass transition point of 50° C. or higher; C represents a divalent group derived from an ethylenic unsaturated monomer which is capable of copolymerizing with the monomers forming both A and B; x represents the fractional content of group A, which ranges from 0.005 to 0.20 mol/mol of polymer of formula (I); y represents the fractional content of group B, which ranges from 0.50 to 0.995 mol/mol of polymer of formula (I); and z represents the fractional content of group C, which ranges from 0 to 0.495 mol/mol of polymer of formula (I).

Formula (II) is represented by



wherein X, Y and Z each represents hydrogen, an alkyl group having from 1 to 6 carbon atoms,  $-COR$  or  $-COOR_1$ ; Q represents



and R represents



where R<sub>1</sub> represents a substituted or an unsubstituted alkyl group having from 1 to 18 carbon atoms, an aryl group having from 6 to 18 carbon atoms, or an aralkyl group having from 7 to 12 carbon atoms; R<sub>2</sub> represents hydrogen, a halogen atom, an alkyl group having from 1 to 12 carbon atoms, or an alkoxy group having from 1 to 6 carbon atoms; R<sub>3</sub> represents hydrogen, a substituted or an unsubstituted alkyl group having from 1 to 4 carbon atoms, a phenyl group or an aralkyl group having from 7 to 10 carbon atoms; R<sub>4</sub> represents the same groups as R<sub>3</sub> or an  $-R_5\text{--CONH}_2\text{--}R_6\text{--COR}_7$  group; R<sub>5</sub> represents a divalent aliphatic or an aromatic group having 1 to 12 carbon atoms, R<sub>7</sub> represents  $-OM$ , hydrogen, a substituted or an unsubstituted alkyl group (C<sub>1</sub>–C<sub>4</sub>), a phenyl group or an aralkyl group (C<sub>7</sub>–C<sub>10</sub>), and l is an integer of 0 to 6; M represents hydrogen or a cation (e.g., an alkali metal atom, an ammonium group, etc.); m is 0 or 1; and n is an integer of 1 to 4.

Formula (III) is represented by



wherein D and E each represents hydrogen, a methyl group, a halogen atom or  $-COOR_6$ ; G represents hydrogen, a methyl group, a halogen atom or  $-(CH_2)_k-COOR_6$ ; J represents hydrogen, an aryl group,



R<sub>6</sub> represents a substituted or an unsubstituted alkyl group having from 1 to 10 carbon atoms, an aryl group having from 6 to 12 carbon atoms or an aralkyl group having from 7 to 12 carbon atoms; and k is 0 or 1.

In another aspect, the present invention relates to a method of forming images comprising imagewise exposing and development-processing a silver halide photographic light-sensitive film material, as described above, wherein the development-processing is carried out using a squeezing means (for example, a rubber lips, squeeze rollers and buff rollers) for removing excess liquid from the film material.

### DETAILED DESCRIPTION OF THE INVENTION

Examples of substituent group which may be present on the alkyl groups, aryl groups and aralkyl groups represented by R<sub>1</sub> or R<sub>6</sub> include a halogen atom (e.g., Cl, Br and F), a cyano group, an alkoxy group having from 1 to 8 carbon atoms, a hydroxy group, a phenoxy group, a dialkylamino group having from 1 to 6 carbon atoms, a furfuryl group, a tetrahydrofurfuryl group, an acyl group having from 1 to 8 carbon atoms, an acyloxy group having from 1 to 8 carbon atoms, a carboalkoxy group having from 1 to 12 carbon atoms, and so on.

Examples of monomers represented by the formula (II) include acrylic acid, methacrylic acid, maleic acid,

monoalkyl maleates (e.g., monomethyl maleate, monoethyl maleate, monobutyl maleate, monoocetyl maleate, monophenyl maleate, etc.), itaconic acid, monoalkyl itaconates (e.g., monomethyl itaconate, monoethyl itaconate, monoocetyl itaconate, etc.), fumaric acid, monoalkyl fumarates (e.g., monomethyl fumarate, monoethyl fumarate, etc.), crotonic acid, methylenemalonic acid, monoalkyl ethylenemalonates (e.g., monomethyl methylenemalonate, monoethyl methylenemalonate, monohexyl methylenemalonate, etc.), citraconic acid,  $\alpha,\beta$ -dimethylmaleate, N-(meth)acryloylamino acids (e.g., N-acryloylglycine, N-methacryloylglycine, N-acryloylglycylglycine, N-methacryloylglycylglycine, N-acryloylalanine, N-methacryloylalanine, N-methacryloylalanylalanine, N-acryloylvaline, N-methacryloylleucine, N-methacryloylisoleucine, N-acryloylproline, N-acryloyl- $\beta$ -aminopropionic acid and N-methacryloyl- $\beta$ -aminopropionic acid), vinylbenzoic acid, acrylamide, N-methylacrylamide, N-hydroxymethylacrylamide, N,N-dimethylacrylamide, N-methoxymethylacrylamide, N-t-butylacrylamide, N,N-diethylacrylamide, methacrylamide, N,N-dimethylmethacrylamide, N,N-diethylmethacrylamide, N-acryloylpiperidine, N-acryloylpiperidine, N-methacryloylmorpholine, N-methacryloylpiperidine, maleic acid monoamide, N-alkylmaleic acid monoamides (e.g., N-ethylmaleic monoamide, N-butylmaleic acid monoamide, etc.), itaconic acid monoamide, N-alkylitaconic acid monoamide (e.g., N-ethylitaconic acid monoamide, N-butylitaconic acid monoamide, etc.), methylenemalonic acid monoamide, N-alkylmethylenemalonic acid monoamides (e.g., N-ethylmethylenemalonic acid monoamide, N-hexylmethylenemalonic acid monoamide, etc.), N,N-dialkylmaleic acid monoamides (e.g., N,N-diethylmaleic acid monoamide, N,N-dibutylmaleic acid monoamide, etc.), N,N-dialkylitaconic acid monoamides (e.g., N,N-diethylitaconic acid monoamide, N,N-dibutylitaconic acid monoamide, etc.) and so on. Therein, the acids may take the form of salt by combining with alkali metals like Na and K, or with ammonium ion.

Examples of monomers represented by the formula (III) include acrylic acid esters, methacrylic acid esters, styrenes, vinyl esters, vinyl ethers, olefins, unsaturated nitriles and so on. These monomers may be employed as the component B in the formula (I), provided that their homopolymers have glass transition points of at least 50° C.

Specific examples of monomers represented by formula (III) whose homopolymers have a glass transition point of at least 50° C. include t-butyl acrylate, isobornyl acrylate, phenyl acrylate, p-chlorophenyl acrylate, methyl methacrylate, ethyl methacrylate, isopropyl methacrylate, t-butyl methacrylate, cyclohexyl methacrylate, cyanoethyl methacrylate, chloroethyl methacrylate, bromoethyl methacrylate, phenyl methacrylate, p-chlorophenyl methacrylate, p-cyanophenyl methacrylate, p-carbomethoxyphenyl methacrylate, p-cyanophenyl methacrylate, adamantly methacrylate, tetrahydrofurfuryl methacrylate, furfuryl methacrylate, isobornyl methacrylate, styrene, methylstyrene,  $\alpha$ -methylstyrene, dimethylstyrene, trimethylstyrene, ethylstyrene, isopropylstyrene, benzylstyrene, chloromethylstyrene, trifluoromethylstyrene, ethoxymethylstyrene, methoxystyrene, chlorostyrene, dichlorostyrene, bromostyrene, fluorostyrene, methyl vinylbenzoate, vinylphenyl acetate, vinyl benzoate, vinyl chlorobenzoate, vinyl naphthoate, t-butyl vinyl ether, isopro-

pyl vinyl ether, isobutyl vinyl ether, phenyl vinyl ether, acrylonitrile, methacrylonitrile, vinyl chloride and so on.

C represents a divalent group derived from an ethylenic unsaturated monomer other than A or B which is capable of copolymerizing with the monomers forming both A and B. For example, acrylic acid esters, methacrylic acid esters, acrylamides, methacrylamides, vinyl esters, vinyl ketones, allyl compounds, olefins, vinyl ethers, N-vinylamides, vinyl heterocyclic compounds, maleic acid esters, itaconic acid esters, fumaric acid esters, crotonic acid esters and so on may be employed as the component C. Specific examples include methyl acrylate, ethyl acrylate, n-propyl acrylate, isopropyl acrylate, n-butyl acrylate, isobutyl acrylate, sec-butyl acrylate, amyl acrylate, hexyl acrylate, 2-ethylhexyl acrylate, octylacrylate, tert-octyl acrylate, 4-chlorobutyl acrylate, cyanoethyl acrylate, dimethylaminoethyl acrylate, cyclohexyl acrylate, 2-hydroxyethyl acrylate, 3-hydroxypropyl acrylate, 2-hydroxypropyl acrylate, 2,3-dihydroxypropyl acrylate, 4-hydroxybutyl acrylate, 5-hydroxypentyl acrylate, 2,2-dimethyl-3-hydroxypropyl acrylate, diethylene glycol monoacrylate, triethylene glycol monoacrylate, dipropylene glycol monoacrylate, glycerol monoacrylate, trimethylolethane monoacrylate, trimethylolpropane monoacrylate, pentaerythritol monoacrylate, 2-methoxyethyl acrylate, 3-methoxybutyl acrylate, 2-ethoxyethyl acrylate, 2-isopropoxyethyl acrylate, 2-butoxyethyl acrylate, 2-(2-methoxyethoxy)ethyl acrylate, 2-(2-butoxyethoxy)ethyl acrylate,  $\omega$ -methoxypolyethylene glycol acrylate (the addition mol number of ethylene oxide groups, "n", is 9 in the formula



$\omega$ -lauroxypolyethylene glycol acrylate (addition mol number n=20), 1-bromo-2-methoxyethyl acrylate, 1,1-dichloro-2-ethoxyethyl acrylate, 2-hydroxy-3-chloropropyl acrylate, amyl methacrylate, hexyl methacrylate, octyl methacrylate, sulfopropyl methacrylate, N,N-diethylaminopropyl methacrylate, 2-hydroxyethyl methacrylate, 3-hydroxypropyl methacrylate, 2-hydroxypropyl methacrylate, 2,3-dihydroxypropyl methacrylate, 4-hydroxybutyl methacrylate, 5-hydroxypentyl methacrylate, 2,2-dimethyl-3-hydroxypropyl methacrylate, diethylene glycol monomethacrylate, dipropylene glycol monomethacrylate, glycerol monomethacrylate, trimethylolethane monomethacrylate, trimethylolpropane monomethacrylate, pentaerythritol monomethacrylate, 2-methoxyethyl methacrylate, 3-methoxybutyl methacrylate, 2-ethoxyethyl methacrylate, 2-isopropoxyethyl methacrylate, 2-butoxyethyl methacrylate, 2-(2-methoxyethoxy)ethyl methacrylate, 2-(2-butoxyethoxy)ethyl methacrylate, 2-(2-butoxyethoxy)ethyl methacrylate,  $\omega$ -methoxypolyethylene glycol methacrylate (addition mol number n=6),  $\omega$ -methoxypolyethylene glycol methacrylate (addition mol number n=23),  $\omega$ -lauroxypolyethylene glycol methacrylate, hexyl acrylamide, octyl acrylamide, 2-acrylamido-2-methylpropanesulfonic acid, N-(1,1-dimethyl-3-oxobutyl)acrylamide, pentyl methacrylamide, dihexyl methacrylamide, allyl caproate, allyl caprate, allyl laurate, allyl palmi-

tate, allyl stearate, allyl acetoacetate, allyl butyrate, allyloxyethanol, allyl butyl ether, hexyl vinyl ether, octyl vinyl ether, decyl vinyl ether, ethylhexyl vinyl ether, methoxyethyl vinyl ether, ethoxyethyl vinyl ether, 2-ethylbutyl vinyl ether, hydroxyethyl vinyl ether, diethylene glycol vinyl ether, dimethylaminoethyl vinyl ether, vinyl formate, vinyl acetate, vinyl propionate, vinyl butyrate, vinyl isobutyrate, vinyl ethyl butyrate, vinyl valerate, vinyl caproate, vinyl methoxacetate, vinyl butoxyacetate, vinyl acetoacetate, vinyl lactate, N-vinylloxazolidone, vinylpyridine, vinylpicoline, N-vinylimidazole, N-vinyl-2-methylimidazole, N-vinyltriazole, N-vinyl-3,5-dimethyltriazole, N-vinylpyrrolidone, N-vinyl-3,5-dimethylpyrazole, N-vinylcarbazole, vinylthiophene, N-vinylsuccinimide, N-vinylglutarimide, N-vinyladipimide, N-methyl-N-vinylformamide, N-ethyl-N-vinylformamide, N-methyl-N-vinylacetamide, N-ethyl-N-vinylacetamide, N-methyl-N-vinylpropionamide, N-vinylpyrrolidone, N-vinylpiperidone, N-vinyl-s-caprolactam, N-vinyl-2-pyridone, vinyl methyl ketone, methoxyethyl vinyl ketone, ethylene, propylene, 1-butene, 1-pentene, 1-hexene, 4-methyl-1-pentene, 1-heptene, 1-octene, 1-decene, 5-methyl-1-nonene, 5,5-dimethyl-1-octene, 4-methyl-1-hexene, 4,4-dimethyl-1-pentene, 5-methyl-1-hexene, 4-methyl-1-heptene, 5-methyl-1-heptene, 4,4-dimethyl-1-hexene, 5,5,6-trimethyl-1-heptene, 1-dodecene, 1-octadecene, dioctyl itaconate, dihexyl itaconate, dibutyl itaconate, maleic anhydride, dihexyl maleate, butyl hexyl maleate, dibutyl maleate, dioctyl maleate, dibutyl fumarate, dioctyl fumarate and so on.

Of these monomers, monomers of the formula (II) wherein X, Y and Z each represents hydrogen,  $-\text{CH}_3$  or  $-\text{COR}$ , and Q represents  $-\text{CH}_2-\text{m}$  are more preferably employed from the viewpoints of the solubilities of the polymers prepared therefrom, the transparencies thereof, the oleophilicities thereof, the hydrophilicities thereof, the affinity thereof for protective colloids (to prevent removal of matting agent from protective colloids, for example, gelatin), the facilities in polymerizations and so on. Particularly, acrylic acid, methacrylic acid, maleic acid, itaconic acid and (meth)acryloylamino acid are preferred therefor. On the other hand, as monomers represented by the formula (III), monomers wherein D and E each represents hydrogen and G represents a methyl group are preferred. Of such monomers, methacrylic acid esters and styrenes are particularly preferable.

In the composition of the polymers of this invention having the formula (I), as the fraction x becomes smaller, the affinity for hydrophilic protective colloids, such as gelatin, becomes weaker. On the other hand, if the fraction x becomes too large, the polymer grains of this invention dissolve in processing solutions for silver halide photographic light-sensitive materials, whereby various disadvantages are caused. Accordingly, the range of x is from 0.005 to 0.20 mol, preferably from 0.01 to 0.18 mol, more preferably from 0.03 to 0.15 mol, and most preferably from 0.03 to less than 0.10 mol, per mol of polymer of formula (I).

Synthesis of these copolymers having repeating units as represented by the formula (I) can be advantageously carried out by reference to the methods as described in British Pat. No. 1,211,039, Japanese Patent Publication No. 29195/72, Japanese Patent Applications Nos. 7174/72, 23466/72, 59743/72 and 31355/73, British Pat. No. 961,395, U.S. Pat. Nos. 3,227,672, 3,290,417, 3,262,919, 3,245,932, 2,681,897 and 3,230,275, John C.

Petropoulos et al., *Official Digest*, Vol. 33, pp. 719-736 (1961), Shunsuke Murahashi et al., Ed., *Gosei Kobunshi* (Synthetic Polymers), Vol. 1, pp. 246-290, and Vol. 3, pp. 1-108, published by Asakura Shoten (1971), and so on. Therein, the polymerization initiator, the concentration, the polymerization temperature, the reaction time and so on can be conveniently varied over a wide range depending upon the end-use purpose.

For instance, polymerization is carried out at a temperature ranging generally from 20° C. to 180° C., and preferably from 40° C. to 120° C. A polymerization reaction is, in general, effected using a radical polymerization initiator in a proportion of from 0.05 to 5 wt% of monomer to be polymerized. As examples of the initiator, mention may be made of azobisis compounds, peroxides, hydroperoxides, redox catalysts and the like. More specifically, they include potassium persulfate, tert-butylperoxyoctoate, benzoyl peroxide, isopropyl percarbonate, 2,4-dichlorobenzoyl peroxide, methyl ethyl ketone peroxide, cumene hydroperoxide, dicumyl peroxide, azobisisobutyronitrile and so on.

Molecular weights of polymers to be employed for the purpose of this invention are generally greater than about 3,000, and preferably they range from 10,000 to 1,000,000 or so. However, these values are not intended to be construed as suggesting critical values for attaining the effects of this invention.

Examples of typical copolymers represented by formula (I) are hereinafter described:

- 
- (1) Acrylic acid-ethyl methacrylate copolymer  
(mol ratio 5/95)  
(2) Acrylic acid-ethyl methacrylate copolymer  
(mol ratio 10/90)  
(3) Acrylic acid-ethyl methacrylate copolymer  
(mol ratio 15/85)  
(4) Methacrylic acid-ethyl methacrylate copolymer  
(mol ratio 18/82)  
(5) Methacrylic acid-methyl methacrylate copolymer  
(mol ratio 10/90)  
(6) Methacrylic acid-methyl methacrylate copolymer  
(mol ratio 15/85)  
(7) Methacrylic acid-methyl methacrylate copolymer  
(mol ratio 5/95)  
(8) Itaconic acid-styrene copolymer  
(mol ratio 5/95)  
(9) Maleic acid-methyl methacrylate copolymer  
(mol ratio 7/93)  
(10) Methacrylic acid-t-butyl acrylate copolymer  
(mol ratio 16:84)  
(11) Acrylic acid-phenyl acrylate copolymer  
(mol ratio 12/88)  
(12) N-Acryloylglycine-t-butyl methacrylate copolymer  
(mol ratio 20/80)  
(13) N-Methacryloylglycine-ethyl methacrylate copolymer  
(mol ratio 14/86)  
(14) Itaconic acid-methyl methacrylate copolymer  
(mol ratio 8/92)  
(15) Maleic acid-styrene copolymer  
(mol ratio 15/85)  
(16) Acrylic acid-i-propyl methacrylate copolymer  
(mol ratio 13/87)  
(17) Acrylic acid-benzyl methacrylate copolymer  
(mol ratio 8/92)  
(18) Acrylic acid-p-chlorophenyl methacrylate copolymer  
(mol ratio 11/89)  
(19) Methacrylic acid-vinyltoluene copolymer  
(mol ratio 13/87)  
(20) Methacrylic acid-n-propyl methacrylate copolymer  
(mol ratio 9/91)  
(21) Fumaric acid-styrene copolymer  
(mol ratio 6/94)  
(22) Acrylic acid-ethyl methacrylate-N-vinylpyrrolidone copolymer (mol ratio 7/85/8)  
(23) Acrylic acid-methacrylic acid-ethyl methacrylate copolymer (mol ratio 5/8/87)

-continued

- (24) Acrylic acid-methyl methacrylate-n-propyl methacrylate copolymer (mol ratio 12/56/32)
- (25) Methacrylic acid-methyl methacrylate-N,N-dimethyl acrylamide copolymer (mol ratio 10/80/10)
- (26) N-Acryloylglycine-ethyl methacrylate-2-hydroxyethyl methacrylate copolymer (mol ratio 10/76/14)
- (27) N-Acryloylglycine-methyl methacrylate-2-hydroxyethyl methacrylate copolymer (mol ratio 8/70/22)
- (28) N-Acryloylglycine-t-butyl methacrylate-N,N-diethylacrylamide copolymer (mol ratio 14/80/6)
- (29) Itaconic acid-ethyl methacrylate-methoxymethyl acrylamide copolymer (mol ratio 7/90/3)
- (30) N-Acryloylglycylglycine-ethyl methacrylate-2-hydroxyethyl methacrylate copolymer (mol ratio 12/72/16)
- (31) Methacrylic acid-ethyl methacrylate-2-hydroxyethyl methacrylate copolymer (mol ratio 10/74/16)
- (32) Methacrylic acid-styrene-chloromethylstyrene copolymer (mol ratio 13/60/27)
- (33) Methacrylic acid-acrylonitrile-butyl methacrylate copolymer (mol ratio 15/60/25)
- (34) Acrylic acid-i-butyl methacrylate-2-acrylamide-2-methylpropanesulfonic acid copolymer (mol ratio 7/89/4)
- (35) Acrylic acid-ethyl methacrylate-N-(1,1-dimethyl-3-oxobutyl)acrylamide copolymer (mol ratio 12/76/12)

An average grain diameter of the matting agent of this invention ranges from  $0.2\mu$  to  $10\mu$ , and preferably from  $1\mu$  to  $8\mu$ .

One of advantages of the matting agent of this invention is that its average grain size is easily controlled in the process of synthesis thereof, based on the factors that the grain size increases as the molecular weight of the polymer and the amount of polymer added are increased, and decreases as the amount of wetting agent used in emulsification is increased.

In this invention, the matting agent is incorporated into the outermost layer of a sensitive material. The outermost layer may be the surface protecting layer, backing layer or both of them. However, it is particularly preferable to allow to incorporate the matting agent in the surface protecting layer.

Another advantage of the matting agent of this invention is that a dissolution tank and the like used in the process of production are washed with ease because the matting agent of this invention which is added to the coating solution for making the outermost layer does not adhere firmly to the wall surfaces of the dissolution tank and the like.

It is desirable in this invention to allow the matting agent to contain an amount of from 2 to 500 mg per square meter of the topmost layer.

In this invention, a binder to constitute the topmost layer is not restricted to particular substance. However, the use of gelatin as a binder is particularly favored.

As for gelatin, any kinds of gelatins, for example, alkali-processed gelatin, acid-processed gelatin, enzyme-processed gelatin, gelatin derivatives and denatured gelatins, are usable, and acid-processed gelatin is the best of these gelatins for purposes of this invention.

Further, the outermost layer of this invention may optionally contain a hardening agent, a smoothing agent, a surface active agent, an antistatic agent, a thickener, polymers, an ultraviolet ray absorbent, a high boiling point solvent, silver halides, a formalin capturing agent, a polymer latex and various other additives.

Examples of a hardening agent employable in this invention include aldehyde series compounds, active halogen-containing compounds such as 2-hydroxy-4,6-dichloro-1,3,5-triazine, vinyl sulfone series compounds,

N-methylol series compounds, halogencarboxyaldehyde compounds such as mucochloric acid, and so on.

Examples of a smoothing agent usable in this invention include liquid paraffins, waxes, polyfluorinated hydrocarbons, silicones, and so on.

As a surface active agent, any kinds of surface active agents, for example, natural surface active agents such as saponin; nonionic surface active agents such as alkyleneoxide series ones; cationic surface active agents such as higher alkylamines, quaternary ammonium salts and so on; anionic surface active agents containing acidic groups such as carboxylic acid, sulfonic acid and so forth. Other known surface active agents can also be employed.

As an antistatic agent, the outermost layer may contain surface active agents as described above, alkali metal salts of styrene-maleic acid series copolymers and acrylonitrile-acrylic acid series copolymers, and antistatic agents as described in U.S. Pat. Nos. 3,206,312, 3,428,451 and so forth.

In addition to the matting agent having a composition represented by formula (I), previously known matting agents can be also employed in this invention. However, these known matting agents are, of course, restricted in their usable amounts to within such a range

that the objects of this invention, viz., (i) that the outermost layer retains satisfactory mat properties even after the completion of development-processing, and (ii) that the matting agent is not removed by being rubbed severely with rubber lips or squeeze rollers, can be attained.

Exemplary useful known matting agents include, for example, a methyl methacrylate (MMA)-methacrylic acid (MA) (molar ratio 5/5) copolymer, MMA-MA (molar ratio range of 6/4 to 9/1) copolymers as described in U.S. Pat. No. 4,142,894; and polymethylmethacrylate (PMMA).

The matting agent PMMA suffers, as described hereinbefore, the disadvantage that it is removed by being rubbed strongly with rubber lips or squeeze rollers.

The matting agent of MMA-MA (5/5) copolymer is soluble to an alkaline developing solution, and, therefore, it cannot provide mat properties after development-processing.

The MMA-MA (6/4 to 9/1) copolymers change their properties sharply depending upon their particular compositions.

Particularly, MMA-MA (6/4 to 7/3) copolymers are soluble in commonly used alkaline developing solutions, while MMA-MA (8/2 to 9/1) copolymers do not have any solubility thereto.

Moreover, the MMA-MA (8/2 to 9/1) copolymers are not removed even by being rubbed strongly with rubber lips or the like.

Although U.S. Pat. No. 4,142,894 broadly discloses MMA-MA copolymers whose compositions extend over a range of molar ratios of from 6/4 to 9/1, only MMA-MA (6/4) copolymer is employed in the Example, and other copolymers are not referred to in the Example.

This invention is characterized by the findings that copolymers having an A-component fraction of from 0.005 to 0.20 mol/mol of polymer of the formula (I) can not be dissolved in alkaline developing solutions, and are not removed by being rubbed severely with rubber lips or the like. Accordingly, the embodiments of the present invention wherein the component A is MA and

the component B is MMA represents a selective invention having unexpected properties in view of the disclosure of U.S. Pat. No. 4,142,894.

This invention does not impose any special restriction on the thickness of the outermost layer. However, it is desirable to adjust the thickness to from  $0.2\mu$  to  $10\mu$ , and particularly to  $1\mu$  to  $8\mu$ .

Embodiments of constituent layers of sensitive materials according to this invention are described below.

Silver halide emulsions can be produced in any conventional manner. For example, a single jet method, a double jet method, a controlled double jet method, an acid process, an ammonia process, or a neutral process may be used for this purpose. Silver halide grains contained in the thus produced emulsion are not restricted in their crystal form, size, and size distribution.

Silver halides which can be preferably employed herein include silver chloride, silver chlorobromide, silver iodobromide, silver chloroiodobromide, and so forth.

As a vehicle for silver halide, not only gelatin, denatured gelatins and gelatin derivatives are employed, but also carboxymethyl cellulose, hydroxyethyl cellulose, starch derivatives, polyvinyl alcohol, poly-N-pyrrolidone, acrylic acid copolymers, polyacrylamides and so on may be used in combination with the above-described gelatins. Moreover, vinyl polymers can be incorporated into photographic layers in the form of a dispersed-in-water type latex. As such latexes, homo- and copolymers of alkyl acrylates, alkyl methacrylates, acrylic acid, methacrylic acid, glycidyl acrylate, styrene, vinyl chloride, vinylidene chloride and the like may be employed.

The silver halide emulsions can be chemically sensitized in a conventional manner. The chemical sensitization can be effected using gold compounds as described in U.S. Pat. Nos. 2,399,083, 2,597,856, etc.; salts of noble metals such as platinum, palladium, rhodium and iridium; sulfur compounds, as described in U.S. Pat. Nos. 2,410,689, 3,501,313, etc.; stannous salts; amines; and so forth.

To the silver halide emulsion of this invention, various compounds can be added which are generally called stabilizers or antifoggants in this art. Specifically, not to speak of 4-hydroxy-6-methyl-1,3,3a,7-tetraazaindene, 3-methylbenzothiazole and 1-phenyl-5-mercaptopotetrazole, various heterocyclic compounds, mercury-containing compounds, mercapto compounds, metal salts and so on can be used therefor.

In addition, various spectral sensitizing dyes, such as 50 merocyanine dyes, carbocyanine dyes, cyanine dyes and the like, can be employed in the silver halide emulsions of this invention depending upon the purpose of the end-use of sensitive materials.

Color couplers which can be employed in this invention include 4-equivalent yellow couplers of diketomethylene series, 2-equivalent yellow couplers of diketomethylene series, 4- or 2-equivalent magenta couplers of pyrazolone series, indazolone series magenta couplers,  $\alpha$ -naphthol series cyan couplers, phenyl series 55 cyan couplers, and the so-called DIR couplers.

Furthermore, dyes, ultraviolet-ray absorbents, hardening agents as described hereinbefore, surface active agents and further, polymer latexes, and other known additives can be incorporated into the silver halide 60 emulsion layers and other photographic layers.

As for supports for the sensitive materials of this invention, materials used conventionally in this art, such

as cellulose acetate film, polyethylene terephthalate film, baryta paper, paper coated with  $\alpha$ -olefin polymers, and so forth, can be employed.

Photographic layers of the sensitive material of this invention can be coated one layer at a time or as multi-layer at a time, using a dip coating technique, an air knife coating technique, a curtain coating technique, an extrusion coating technique, or other known technique.

Selection of various additives, vehicle, a support, a coating method and so on which are to be employed in this invention can be done by reference to the description in *Research Disclosure*, Vol. 176, pp. 22-31 (Dec., 1978).

As sensitive materials which can be prepared in accordance with embodiments of this invention, mention may be made of color negative films, color reversal films, color paper, motion picture color negative films, color positive films, X-ray films, films for making printing plates, and so forth.

20 A light source for exposing the sensitive material thereto does not receive any restrictions in its illumination intensity and so on. Exposure is generally continued for from about 10 to  $10^{-6}$  sec.

After exposure, the sensitive material of this invention is subjected to a development-processing in order to produce a silver image and/or dye image.

Any of known processes can be applied to photographic processings of the sensitive material of this invention. Therein, known processing solutions can be used. The processing temperature is commonly selected from the range of from 18° C. to 50° C. However, a temperature below 18° C. or above 50° C. may be employed as the processing temperature. Either a development-processing for producing a silver image (black-and-white photographic processing) or a color photographic processing including the development-processing for producing dye images may be applied to this invention, depending upon the purpose of the end-use of the sensitive material.

A developing solution to be employed in the case of black-and-white photographic processing can contain known developing agents. As such a developing agent, dihydroxybenzenes (e.g., hydroquinone); 3-pyrazolidones (e.g., 1-phenyl-3-pyrazolidone); aminophenols (e.g., N-methyl-p-aminophenol); 1-phenyl-3-pyrazolines; ascorbic acid; such heterocyclic compounds as to be produced by condensing a 1,2,3,4-tetrahydroquinoline ring and an indolene ring, as described in U.S. Pat. No. 4,067,872; and so on can be employed independently or in combination thereof. In addition to these developing agents, a developing solution may generally contain known preservatives, alkali agents, pH buffers and antifoggants, and further it may optionally contain dissolving aids, color toning agents, development accelerators, surface active agents, defoaming agents, water softeners, hardening agents, viscosity providing agents and so on.

To the sensitive material of this invention, the so-called "lithographic" development-processing can be applied. The term "lithographic" development-processing describes the development-processing of the kind in which development is made to proceed infectiously by the use of dihydroxybenzenes as a developing agent in the presence of a low concentration of sulfite ion with the intention of photographically reproducing line images, or half tone images utilizing half tone dots, which is described in detail in L.F.A. Mason, *Photographic Processing Chemistry*, pp. 163-165 (1966).

As a fixing solution, those compositions which have conventionally been used can be used in this invention also.

As the fixing agent, thiosulfates, thiocyanates, and organic sulfur compounds which have been known to be effective as a fixing agent can be employed.

These fixing solutions may contain water-soluble aluminum salts as a hardening agent.

Conventional methods can be applied to this invention upon the production of dye images. Namely, the negative-positive method, as described, e.g., in *Journal of the Society of Motion Picture and Television Engineers*, Vol. 61, pp. 667-701 (1953); the color reversal process, in which, to begin with, a negative silver image is produced through development using a black-and-white developing agent and then overall exposure is undertaken at least once, or another appropriate uniform fogging treatment is carried out and subsequently, color development is effected to produce positive dye image; and silver dye bleach process in which silver image is produced by the development of dye-containing photographic emulsion layers after exposure, and dyes are bleached using the resulting silver image as a bleaching catalyst; and so on can be applied.

Color developing solutions generally include alkaline aqueous solutions containing color developing agents. As color developing agents, known aromatic primary amine developers, such as phenylenediamines (e.g., 4-amino-N,N-diethylaniline, 3-methyl-4-amino-N,N-diethylaniline, 4-amino-N-ethyl-N-β-hydroxyethylaniline, 3-methyl-4-amino-N-ethyl-N-β-hydroxyethylaniline, 3-methyl-4-amino-N-ethyl-N-β-methanesulfonamidoethylaniline, 4-amino-3-methyl-N-ethyl-N-β-methoxyethylaniline, etc.), can be used.

In addition to these color developing agents, those which are described in L.F.A. Mason, *Photographic Processing Chemistry*, pp. 226-229, Focal Press (1966), U.S. Pat. Nos. 2,193,015 and 2,592,364, Japanese Patent Application (OPI) 64933/73 (the term "OPI" as used herein refers to a "published unexamined Japanese patent application"), and so forth may be also employed.

The color developing solutions may additionally contain pH buffers such as the sulfites, the carbonate and the phosphates of alkali metals; development restrainers or antifogging agents such as bromides, iodides and organic antifogging agents; and so on. Further, water softeners, preservatives such as hydroxyamine, organic solvents such as benzyl alcohol and diethylene glycol, development accelerators such as polyethylene glycol, quaternary ammonium salts and amines, dye forming couplers, competing couplers, fogging agents such as sodium borohydride, assistant developers such as 1-phenyl-3-pyrazolidone, viscosity providing agents, chelating agents of polycarboxylic acid series as described in U.S. Pat. No. 4,083,723; antioxidants as described in German Patent Application (OLS) No. 2,622,950; and so on may be optionally contained in the color developing solutions.

After color development, the photographic emulsion layers are generally subjected to a bleaching processing. The bleaching processing may be carried out simultaneously with a fixing processing, or it may be carried out individually. Examples of bleaching agents employable in the bleaching processing include compounds of multivalent metals such as Fe(III), Co(III), Cr(IV), Cu(II), etc., peroxy acids, quinones, nitroso compounds and so on. More specifically, ferricyanides, dichromates; organic complex salts of Fe(III) or Co(III), for example, the complex salts of organic acids such as aminopolycarboxylic acids (e.g., ethylenediaminetetraacetic acid, nitrilotriacetic acid, 1,3-diamino-2-propanoltetraacetic acid, etc.), citric acid, tartaric acid, malic acid and so on; persulfates; permanganates; nitrosophenol; and so on can be used. Among these bleaching agents, potassium ferricyanide, sodium ethylenediaminetetraacetatoferate(III), and ammonium ethylenediaminetetraacetatoferate(III) are particularly useful. Especially, ethylenediaminetetraacetatoiron(III) complex salts are useful in both an independent bleaching solution and a combined bleaching and fixing bath.

To a bleaching solution or a combined bleaching and fixing bath, bleaching accelerators as described in U.S. Pat. Nos. 3,042,520 and 3,241,966, Japanese Patent Publications Nos. 8506/70 and 8836/70, and so on; thiol compounds as described in Japanese Patent Application (OPI) No. 65732/78, and other additives can be also added.

The sensitive materials prepared in accordance with embodiments of this invention may be processed with the developing solutions which are replenished or controlled so as to maintain their developabilities by such means as described in Japanese Patent Applications (OPI) Nos. 84636/76, 11934/77, 46732/78, 9626/79, 19741/79 and 37731/79, and Japanese Patent Applications Nos. 76159/79 and 102962/79.

Bleach-fix baths regenerated by such means as described in Japanese Patent Applications (OPI) Nos. 781/71, 49437/73, 18191/73, 145231/75, 18541/76, 19535/76 and 144620/76, and Japanese Patent Publication 23178/76 may be applied to the sensitive materials prepared in accordance with embodiments of this invention.

The present invention will now be illustrated in greater detail by reference to the following example.

#### EXAMPLE

Samples 1 to 10 were prepared by providing on their respective supports, which were made of a cellulose triacetate film having a subbing layer, the same red-sensitive emulsion layers, the same interlayers, the same green-sensitive emulsion layers, the same yellow filter layers, the same blue-sensitive emulsion layers and different outermost layers in order of description.

Embodiments of these layers, other than the outermost layers, are summarized in the following Table 3.

The formulae of the outermost layers are shown in 60 the following Table 1.

TABLE 1

| Sample No. | Composition | Formula of Outermost Layer |                      |                                    |                          |
|------------|-------------|----------------------------|----------------------|------------------------------------|--------------------------|
|            |             | Matting Agent              | Average Diameter (μ) | Amount Coated (mg/m <sup>2</sup> ) | Other Additives (common) |
| 1          | PMMA        |                            | 3.5                  | 20                                 | Gelatin                  |

TABLE 1-continued

| Sample No.      | Composition        | Matting Agent              |                                    |                                  |
|-----------------|--------------------|----------------------------|------------------------------------|----------------------------------|
|                 |                    | Average Diameter ( $\mu$ ) | Amount Coated (mg/m <sup>2</sup> ) | Other Additives (common)         |
| (Comparison) 2  | PMMA               | 3.5                        | 120                                | 1.0 g/m <sup>2</sup>             |
| (Comparison) 3  | MMA:MA = 95:5      | 3.5                        | 20                                 | Sodium Dodecyl-benzene-sulfonate |
| (Invention) 4   | MMA:MA = 95:5      | 3.5                        | 120                                | 15 mg/m <sup>2</sup>             |
| (Invention) 5   | MMA:MA = 90:10     | 3.5                        | 20                                 |                                  |
| (Invention) 6   | MMA:MA = 90:10     | 3.5                        | 120                                |                                  |
| (Invention) 7   | MMA:MA = 85:15     | 3.5                        | 20                                 |                                  |
| (Invention) 8   | EMA:MA:AA = 87:8:5 | 3.5                        | 20                                 |                                  |
| (Invention) 9   | MMA:MA = 60:40     | 3.5                        | 20                                 |                                  |
| (Comparison) 10 | MMA:MA = 75:25     | 3.5                        | 20                                 |                                  |
| (Comparison)    |                    |                            |                                    |                                  |

EMA: Ethyl Methacrylate

AA: Acrylic Acid

Each of the thus prepared samples was cut in the form of strip having a width of 35 mm and a length of about 100 m, and subjected to color development processes.

A developing solution used was that which was prepared according to the ECN-II formula (opened formula by Eastmen Kodak Co.), a developing temperature was 38° C., and the sample conveying speed was 21 m/min.

An automatic developing machine used was Pako Cine/Strip Processor Model 35-17 ECN II (produced by Pako Ltd.).

A rubber lips made of silicone rubber was arranged just behind the last processing bath. The rubber lip had such a shape that its width was 40 mm, its thickness was 8 mm, and its tip was cut at an acute angle. The rubber lips was so designed that two lips were in a tip-to-tip contact, and samples were made to pass therethrough.

After the processing of an approximately 33 m portion of each sample, the extent of removal of matting agent due to passage through the rubber lips and a mat property of the processed sample were examined, and compared with one another. The results obtained are shown in Table 2.

#### (i) Removal Test of Matting Agent

The extent of removal was evaluated by the number of aggregated particles adhering to the sample (35 mm wide and 30 m long), which aggregated particles were formed by the matting agent removal due to passage through the rubber lips.

| Rank | Number of Condensates Adhered to Sample |
|------|-----------------------------------------|
| A    | 0                                       |
| B    | 5 or less                               |
| C    | 6-25                                    |
| D    | 26-100                                  |
| E    | 101 or more                             |

#### (ii) Mat Property after Processings

The surface of each processed sample was observed under a microscope, and examined whether the matting agent was retained in its original form (the same form as it had before development processing) or not; whether

30 the matting agent was dissolved away or not; and whether the matting agent was deformed or not.

As can be seen from Table 2, the samples 3 to 8 prepared in accordance with embodiments of this invention did not show removal of their respective matting agents, and retained good mat property even after the completion of development-processing.

On the other hand, in each of samples 1 and 2 where PMMA was employed as the matting agent, the matting agent was removed by the rubber lips and adhered again to other parts of the sample. Therefore, the quality of the processed material was spoiled to a great extent.

In addition, in the cases of the samples 9 and 10 where the MMA-MA (60:40) copolymer and the MMA-MA (75:25) copolymer were employed respectively, whole or a large portion of the matting agent was dissolved into the processing solution. Consequently, the processed materials lost their original mat properties completely.

TABLE 2

| Sample No.        | Removal Test    | Mat Property after Processings                                                     |
|-------------------|-----------------|------------------------------------------------------------------------------------|
| 1<br>(Comparison) | D               | Each grains in the aggregated particles <sup>*1</sup> retained their original form |
| 2<br>(Comparison) | E               | Each grains in the aggregated particles <sup>*1</sup> retained their original form |
| 3<br>(Invention)  | A               | Grains are present as they were initially.                                         |
| 4<br>(Invention)  | A               | Grains are present as they were initially.                                         |
| 5<br>(Invention)  | A               | Grains are present as they were initially.                                         |
| 6<br>(Invention)  | A               | Grains are present as they were initially.                                         |
| 7<br>(Invention)  | A               | Grains are present as they were initially.                                         |
| 8<br>(Invention)  | A               | Grains are present as they were initially.                                         |
| 9<br>(Comparison) | A <sup>*2</sup> | Almost all grains were removed.                                                    |
| 10                | A <sup>*2</sup> | A small number of deformed                                                         |

TABLE 2-continued

| Sample No.   | Test | Mat Property after Processings |
|--------------|------|--------------------------------|
| (Comparison) |      | grains remained.               |

\*<sup>1</sup>Matting agent was removed by the rubber lips and the removed matting agent grains were aggregated to form aggregated particles and, the aggregated particles adhered again to other parts of the sample.

\*<sup>2</sup>whole or a large portion of the matting agent was dissolved into the processing solution and, therefore, no adhered aggregated particle was observed.

ethyl acrylate, n-propyl acrylate, isopropyl acrylate, n-butyl acrylate, isobutyl acrylate, sec-butyl acrylate, amyl acrylate, hexyl acrylate, 2-ethylhexyl acrylate, octylacrylate, tert-octyl acrylate, 4-chlorobutyl acrylate, cyanoethyl acrylate, dimethylaminoethyl acrylate, cyclohexyl acrylate, 2-hydroxyethyl acrylate, 3-hydroxypropyl acrylate, 2-hydroxypropyl acrylate, 2,3-dihydroxypropyl acrylate, 4-hydroxybutyl acrylate, 5-hydroxypentyl acrylate, 2,2-dimethyl-3-hydroxypro-

TABLE 3

|                     | Red-Sensitive Emulsion Layer                                   | Green-Sensitive Emulsion Layer                                                         | Blue-Sensitive Emulsion Layer                                                | Interlayer              | Yellow Filter Layer             |
|---------------------|----------------------------------------------------------------|----------------------------------------------------------------------------------------|------------------------------------------------------------------------------|-------------------------|---------------------------------|
| Color Forming Agent | 4-Chloro-1-hydroxy-N—dodecyl-2-naphthamide                     | 1-(2,4,6-Trichlorophenyl)-3-[3-(2,4-di-t-amylphenoxy)-acetamido]benzamido-5-pyrazolone | 3-(2,4-Di-t-amyl-phenoxyacetamido)- $\alpha$ -(4-methoxybenzoyl)-acetanilide | —                       | —                               |
|                     | 0.88 g/m <sup>2</sup>                                          | 0.75 g/m <sup>2</sup>                                                                  | 1.31 g/m <sup>2</sup>                                                        |                         |                                 |
| Spectral Sensitizer | Bis(9-ethyl-5-phenyl-5-                                        | —                                                                                      | —                                                                            | —                       | —                               |
| Sensitizer          | chloro-3- $\beta$ -hydroxyethyl)thiacarbocyanine Bromide       | 3-ethyl)oxycarbocyanine Isothiocyanate                                                 |                                                                              |                         |                                 |
|                     | 6.51 mg/m <sup>2</sup>                                         | 5.23 mg/m <sup>2</sup>                                                                 |                                                                              |                         |                                 |
| Stabilizer          | 5-Hydroxy-7-methyl-1,3,8-triazaindolidine                      | The same as at the left                                                                | The same as at the left                                                      | —                       | —                               |
|                     | 8.19 mg/m <sup>2</sup>                                         | 7.71 mg/m <sup>2</sup>                                                                 | 6.50 mg/m <sup>2</sup>                                                       |                         |                                 |
| Hardener            | 2,4-Dichloro-6-hydroxy-1,3,5-triazine Sodium Salt              | The same as at the left                                                                | The same as at the left                                                      | The same as at the left | The same as at the left         |
|                     | 15 mg/m <sup>2</sup>                                           | 14 mg/m <sup>2</sup>                                                                   | 20 mg/m <sup>2</sup>                                                         | 10 mg/m <sup>2</sup>    | 11 mg/m <sup>2</sup>            |
| Coating Aids        | Sodium p-Dodecylbenzenesulfonate                               | The same as at the left                                                                | The same as at the left                                                      | The same as at the left | The same as at the left         |
|                     | 42 mg/m <sup>2</sup>                                           | 51 mg/m <sup>2</sup>                                                                   | 67 mg/m <sup>2</sup>                                                         | 56 mg/m <sup>2</sup>    | 63 mg/m <sup>2</sup>            |
|                     | Sodium p-Nonyl-phenoxypoly(ethyleneoxy)-propanesulfonate       | The same as at the left                                                                | The same as at the left                                                      | The same as at the left | The same as at the left         |
|                     | 53 mg/m <sup>2</sup>                                           | 64 mg/m <sup>2</sup>                                                                   | 84 mg/m <sup>2</sup>                                                         | 71 mg/m <sup>2</sup>    | 80 mg/m <sup>2</sup>            |
|                     |                                                                | 64 mg/m <sup>2</sup>                                                                   | 84 mg/m <sup>2</sup>                                                         | 71 mg/m <sup>2</sup>    | 80 mg/m <sup>2</sup>            |
|                     | Silver iodobromide emulsion (silver iodide content: 5.5 mol %) |                                                                                        |                                                                              |                         |                                 |
| Dry                 | 5 $\mu$                                                        | 6 $\mu$                                                                                | 5 $\mu$                                                                      | 2 $\mu$                 | Yellow colloidal silver 2 $\mu$ |

While the invention has been described in detail and with reference to specific embodiments thereof, it will be apparent to one skilled in the art that various changes and modifications can be made therein without departing from the spirit and scope thereof.

What is claimed is:

1. A silver halide photographic light-sensitive material which has on a support at least one light-sensitive silver halide emulsion layer, said material containing in its outermost layer at least one kind of alkali-insoluble synthetic polymer grains having a glass transition point of at least 60° C. and an average grain size of from 0.2 $\mu$  to 10 $\mu$ , and said polymer is represented by formula (I)



wherein A represents a divalent group derived from at least one monomer having the formula (II); B represents a divalent group derived from at least one monomer having the formula (III), whose homopolymer has a glass transition point of at least 50° C.; C represents a divalent group derived from an ethylenic unsaturated monomer other than A or B which is capable of copolymerizing with the monomers forming both A and B, said divalent group being derived from a member selected from the group consisting of methyl acrylate,

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8

pane monomethacrylate, pentaerythritol monomethacrylate, 2-methoxyethyl methacrylate, 3-methoxybutyl methacrylate, 2-ethoxyethyl methacrylate, 2-isopropoxymethyl methacrylate, 2-butoxyethyl methacrylate, 2-(2-methoxyethoxy)ethyl methacrylate, 2-(2-ethoxyethoxy)ethyl methacrylate, 2-(2-butoxyethoxy)ethyl methacrylate,  $\omega$ -methoxypolyethylene glycol methacrylate wherein the addition mol number of ethylene oxide groups is 6,  $\omega$ -methoxypolyethylene glycol methacrylate wherein the addition mol number of ethylene oxide groups is 23,  $\omega$ -lauroxypolyethylene glycol methacrylate, hexyl acrylamide, octyl acrylamide, 2-acrylamido-2-methylpropane-sulfonic acid, N-(1,1-dimethyl-3-oxobutyl)acrylamide, pentyl methacrylamide, dihexyl methacrylamide, allyl caproate, allyl caprate, allyl laurate, allyl palmitate, allyl stearate, allyl acetoacetate, allyl butyrate, allyloxyethanol, allyl butyl ether, hexyl vinyl ether, octyl vinyl ether, decyl vinyl ether, ethyl-hexyl vinyl ether, methoxyethyl vinyl ether, ethoxyethyl vinyl ether, 2-ethylbutyl vinyl ether, hydroxyethyl vinyl ether, diethylene glycol vinyl ether, dimethylaminoethyl vinyl ether, vinyl formate, vinyl acetate, vinyl propionate, vinyl butyrate, vinyl isobutyrate, vinyl ethyl butyrate, vinyl valerate, vinyl caproate, vinyl methoxyacetate, vinyl butoxyacetate, vinyl acetooacetate, vinyl lactate, N-vinyloxazolidone, vinylpyridine, vinylpicoline, N-vinylimidazole, N-vinyl-2-methylimidazole, N-vinyl-triazole, N-vinyl-3,5-dimethyltriazole, N-vinyl, pyrrolidone, N-vinyl-3,5-dimethylpyrazole, N-vinylcarbazole, vinylthiophene, N-vinylsuccinimide, N-vinylglutarimide, N-vinylalldipimide, N-methyl-N-vinylformamide, N-ethyl-N-vinylformamide, N-methyl-N-vinylacetamide, N-ethyl-N-vinylacetamide, N-methyl-N-vinylpropionamide, N-vinylpyrrolidone, N-vinylpiperidone, N-vinyl-s-caprolactam, N-vinyl-2-pyridone, vinyl methyl ketone, methoxyethyl vinyl ketone, ethylene, propylene, 1-butene, 1-pentene, 1-hexene, 4-methyl-1-pentene, 1-heptene, 1-octene, 1-decene, 5-methyl-1-nonene, 5,5-dimethyl-1-octene, 4-methyl-1-hexene, 4,4-dimethyl-1-pentene, 5-methyl-1-hexene, 4-methyl-1-heptene, 5-methyl-1-heptene, 4,4-dimethyl-1-hexene, 5,5,6-trimethyl-1-heptene, 1-dodecene, 1-octadecene, dioctyl itaconate, dihexyl itaconate, dibutyl itaconate, maleic anhydride, dihexyl maleate, butyl hexyl maleate, dibutyl maleate, dioctyl maleate, dibutyl fumarate, and dioctyl fumarate; x represents the fractional content of group A, which ranges from 0.03 to less than 0.1 mol/mol of polymer of formula (I); y represents the fractional content of group B, which ranges from 0.50 to 0.97 mol/mol of polymer of formula (I); and z represents the fractional content of group C, which ranges from 0 to 0.47 mol/mol of polymer of formula (I), and formula (II) is represented by



wherein X, Y and Z each represents hydrogen, an alkyl group having from 1 to 6 carbon atoms, —COR, or —COOR<sub>1</sub>; Q represents



and  $R$  represents



15 where  $R_1$  represents a substituted or an unsubstituted alkyl group having from 1 to 18 carbon atoms, an aryl group having from 6 to 18 carbon atoms, or an aralkyl group having from 7 to 12 carbon atoms;  $R_2$  represents hydrogen, a halogen atom, an alkyl group having from 1 to 12 carbon atoms or an alkoxy group having from 1 to 6 carbon atoms;  $R_3$  represents hydrogen, a substituted or an unsubstituted alkyl group having from 1 to 4 carbon atoms, a phenyl group or an aralkyl group having from 7 to 10 carbon atoms;  $R_4$  represents the same groups as  $R_3$  or an  $-R_5-\text{CONH}R_6-\text{COR}_7$  group, wherein  $R_5$  represents a divalent aliphatic or an aromatic group ( $C_1-C_{12}$ ),  $R_7$  represents  $-\text{OM}$ , hydrogen, a substituted or an unsubstituted alkyl group ( $C_1-C_4$ ), a phenyl group or an aralkyl group ( $C_7-C_{10}$ ), and  $l$  is an integer of 0 to 6;  $M$  represents hydrogen or a cation;  $m$  is 0 or 1; and  $n$  is an integer of from 1 to 4; and formula (III) is represented by



40 wherein D and E each represents hydrogen, a methyl group, a halogen atom, or  $-\text{COOR}_6$ ; G represents hydrogen, a methyl group, a halogen atom or  $-(\text{CH}_2-)_k-\text{COOR}_6$ ; J represents hydrogen, an aryl group,



R<sub>6</sub> represents a substituted or an unsubstituted alkyl group having from 1 to 10 carbon atoms, an aryl group having from 6 to 12 carbon atoms, or an aralkyl group having from 7 to 12 carbon atoms; and k is 0 or 1.

2. A silver halide photographic light-sensitive material as in claim 1, wherein said divalent group A is represented by the formula (II) wherein X, Y and Z each is 55  $\text{CO}_2\text{Hydrogen}$ , and a is  $\text{--} \text{CH}_2 \text{CH}_2 \text{--}$ .

3. A silver halide photographic light-sensitive material as in claim 1, wherein said formula (II) represents 60 acrylic acid, methacrylic acid, maleic acid, itaconic acid or acryloylamino acid.

4. A silver halide photographic light-sensitive material as in claim 3, wherein said formula (II) represents acrylic acid or methacrylic acid.

65 5. A silver halide photographic light-sensitive material as in claim 1, wherein said monomer B is represented by the formula (III) wherein D and E each is hydrogen and G is a methyl group.

6. A silver halide photographic light-sensitive material as in claim 1, wherein said formula (III) represents a methacrylic acid ester or a styrene.

7. A silver halide photographic light-sensitive material as in claim 1, wherein said formula (II) represents acrylic acid or methacrylic acid, and said formula (III) represents a methacrylic acid ester or a styrene.

8. A silver halide photographic light-sensitive material as in claim 7, wherein z in said formula (I) is zero.

9. A silver halide photographic light-sensitive material as in claim 1, 2, 3, 4, 5, 6, 7, or 8, wherein said outermost layer is a surface protecting layer, and said polymer grains are coated in an amount of from 2 to 500 mg per square meter.

10. A silver halide photographic light-sensitive material as in claim 1, 2, 3, 4, 5, 6, 7, or 8, wherein the average grain diameter of the polymeric grains is from  $1\mu$  to  $8\mu$ .

11. A method for forming photographic images comprising imagewise exposing and development-processing a silver halide photographic sensitive material wherein during said development-processing excess liquid is removed from the film material surface by squeezing means, wherein said silver halide photographic light-sensitive material has on a support at least one light-sensitive silver halide emulsion layer, said material containing in its outermost layer at least one kind of alkali insoluble synthetic polymer grains having a glass transition point of at least  $60^\circ\text{C}$ . and an average grain size of from  $0.2\mu$  to  $10\mu$ , and said polymer is represented by formula (I)



(I)

wherein A represents a divalent group derived from at least one monomer having the formula (II); B represents a divalent group derived from at least one monomer having the formula (III), whose homopolymer has a glass transition point of at least  $50^\circ\text{C}$ ; C represents a divalent group derived from an ethylenic unsaturated monomer other than A or B which is capable of copolymerizing with the monomers forming both A and B, said divalent group being derived from a member selected from the group consisting of methyl acrylate, ethyl acrylate, n-propyl acrylate, isopropyl acrylate, n-butyl acrylate, isobutyl acrylate, sec-butyl acrylate, amyl acrylate, hexyl acrylate, 2-ethylhexyl acrylate, octylacrylate, tert-octyl acrylate, 4-chlorobutyl acrylate, cyanoethyl acrylate, dimethylaminoethyl acrylate, cyclohexyl acrylate, 2-hydroxyethyl acrylate, 3-hydroxypropyl acrylate, 2-hydroxypropyl acrylate, 2,3-dihydroxypropyl acrylate, 4-hydroxybutyl acrylate, 5-hydroxypentyl acrylate, 2,2-dimethyl-3-hydroxypropyl acrylate, diethylene glycol monoacrylate, triethylene glycol monoacrylate, dipropylene glycol monoacrylate, glycerol monoacrylate, trimethylolethane monoacrylate, trimethylolpropane monoacrylate, pentaerythritol monoacrylate, 2-methoxyethyl acrylate, 3-methoxybutyl acrylate, 2-ethoxyethyl acrylate, 2-isopropoxyethyl acrylate, 2-butoxyethyl acrylate, 2-(2-methoxyethoxy)ethyl acrylate, 2-(2-ethoxyethoxy)ethyl acrylate, 2-(2-butoxyethoxy)ethyl methacrylate,  $\omega$ -methoxypolyethylene glycol methacrylate wherein the addition mol number of ethylene oxide groups is 6,  $\omega$ -methoxypolyethylene glycol methacrylate wherein the addition mol number of ethylene oxide groups is 23,  $\omega$ -lauroxypolyethylene glycol methacrylate wherein the addition mol number of ethylene oxide groups is 20, hexyl acrylamide, octyl acrylamide, 2-acrylamido-2-methylpropanesulfonic acid, N-(1,1-dimethyl-3-oxobutyl)acrylamide, pentyl methacrylamide, dihexyl methacrylamide, allyl caproate, allyl caprate, allyl laurate, allyl palmitate, allyl stearate, allyl acetoacetate, allyl butyrate, allyloxyethanol, allyl butyl ether, hexyl vinyl ether, octyl vinyl ether, decyl vinyl ether, ethylhexyl vinyl ether, methoxyethyl vinyl ether, ethoxyethyl vinyl ether, 2-ethylbutyl vinyl ether, hydroxyethyl vinyl ether, diethylene glycol vinyl ether, dimethylaminoethyl vinyl ether, vinyl formate, vinyl acetate, vinyl propionate, vinyl butyrate, vinyl isobutyrate, vinyl ethyl butyrate, vinyl valerate, vinyl caproate, vinyl methoxyacetate, vinyl butoxyacetate, vinyl acetoacetate, vinyl lactate, N-vinyloxazolidone, vinylpyridine, vinylpicoline, N-vinylimidazole, N-vinyl-2-methylinimidazole, N-vinyl-triazole, N-vinyl-3,5-dimethyltriazole, N-vinyl, pyrrolidone, N-vinyl-3,5-dimethylpyrazole, N-vinylcarbazole, vinylthiophene, N-vinylsuccinimide, N-vinylglutarimide, N-vinyladipimide, N-methyl-N-vinylformamide, N-ethyl-N-vinylformamide, N-methyl-N-vinylacetamide, N-ethyl-N-vinylacetamide, N-methyl-N-vinylpropionamide, N-vinylpyrrolidone, N-vinylpiperidone, N-vinyl-scaprolactam, N-vinyl-2-pyridone, vinyl methyl ketone, methoxyethyl vinyl ketone, ethylene, propylene, 1-butene, 1-pentene, 1-hexene, 4-methyl-1-pentene, 1-heptene, 1-octene, 1-decene, 5-methyl-1-nonene, 5,5-dimethyl-1-octene, 4-methyl-1-hexene, 4,4-dimethyl-1-pentene, 5-methyl-1-hexene, 4-methyl-1-heptene, 5-methyl-1-heptene, 4,4-dimethyl-1-hexene, 5,5,6-trimethyl-1-heptene, 1-dodecene, 1-octadecene, diethyl itaconate, dihexyl itaconate, dibutyl itaconate, maleic anhydride, dihexyl maleate, butyl hexyl maleate, dibutyl maleate, diethyl maleate, dibutyl fumarate, and diethyl fumarate; x represents the fractional content of group A, which ranges from 0.03 to less than 0.1 mol/mol of polymer of formula (I); y represents the fractional content of group B, which ranges from 0.50 to 0.97 mol/mol of polymer of formula (I); and z represents the fractional content of group C, which ranges from 0 to 0.47 mol/mol of polymer of formula (I), and formula (II) is represented by

N,N-diethylaminopropyl methacrylate, 2-hydroxyethyl methacrylate, 3-hydroxypropyl methacrylate, 2-hydroxypropyl methacrylate, 2,3-dihydroxypropyl methacrylate, 4-hydroxybutyl methacrylate, 5-hydroxypentyl methacrylate, 2,2-dimethyl-3-hydroxypropyl methacrylate, diethylene glycol monomethacrylate, triethylene glycol monomethacrylate, dipropylene glycol monomethacrylate, glycerol monomethacrylate, trimethylolethane monomethacrylate, trimethylolpropane monomethacrylate, pentaerythritol monomethacrylate, 2-methoxyethyl methacrylate, 3-methoxybutyl methacrylate, 2-ethoxyethyl methacrylate, 2-isopropoxyethyl methacrylate, 2-butoxyethyl methacrylate, 2-(2-methoxyethoxy)ethyl methacrylate, 2-(2-ethoxyethoxy)ethyl methacrylate, 2-(2-butoxyethoxy)ethyl methacrylate,  $\omega$ -methoxypolyethylene glycol methacrylate wherein the addition mol number of ethylene oxide groups is 6,  $\omega$ -methoxypolyethylene glycol methacrylate wherein the addition mol number of ethylene oxide groups is 23,  $\omega$ -lauroxypolyethylene glycol methacrylate wherein the addition mol number of ethylene oxide groups is 20, hexyl acrylamide, octyl acrylamide, 2-acrylamido-2-methylpropanesulfonic acid, N-(1,1-dimethyl-3-oxobutyl)acrylamide, pentyl methacrylamide, dihexyl methacrylamide, allyl caproate, allyl caprate, allyl laurate, allyl palmitate, allyl stearate, allyl acetoacetate, allyl butyrate, allyloxyethanol, allyl butyl ether, hexyl vinyl ether, octyl vinyl ether, decyl vinyl ether, ethylhexyl vinyl ether, methoxyethyl vinyl ether, ethoxyethyl vinyl ether, 2-ethylbutyl vinyl ether, hydroxyethyl vinyl ether, diethylene glycol vinyl ether, dimethylaminoethyl vinyl ether, vinyl formate, vinyl acetate, vinyl propionate, vinyl butyrate, vinyl isobutyrate, vinyl ethyl butyrate, vinyl valerate, vinyl caproate, vinyl methoxyacetate, vinyl butoxyacetate, vinyl acetoacetate, vinyl lactate, N-vinyloxazolidone, vinylpyridine, vinylpicoline, N-vinylimidazole, N-vinyl-2-methylinimidazole, N-vinyl-triazole, N-vinyl-3,5-dimethyltriazole, N-vinyl, pyrrolidone, N-vinyl-3,5-dimethylpyrazole, N-vinylcarbazole, vinylthiophene, N-vinylsuccinimide, N-vinylglutarimide, N-vinyladipimide, N-methyl-N-vinylformamide, N-ethyl-N-vinylformamide, N-methyl-N-vinylacetamide, N-ethyl-N-vinylacetamide, N-methyl-N-vinylpropionamide, N-vinylpyrrolidone, N-vinylpiperidone, N-vinyl-scaprolactam, N-vinyl-2-pyridone, vinyl methyl ketone, methoxyethyl vinyl ketone, ethylene, propylene, 1-butene, 1-pentene, 1-hexene, 4-methyl-1-pentene, 1-heptene, 1-octene, 1-decene, 5-methyl-1-nonene, 5,5-dimethyl-1-octene, 4-methyl-1-hexene, 4,4-dimethyl-1-pentene, 5-methyl-1-hexene, 4-methyl-1-heptene, 5-methyl-1-heptene, 4,4-dimethyl-1-hexene, 5,5,6-trimethyl-1-heptene, 1-dodecene, 1-octadecene, diethyl itaconate, dihexyl itaconate, dibutyl itaconate, maleic anhydride, dihexyl maleate, butyl hexyl maleate, dibutyl maleate, diethyl maleate, dibutyl fumarate, and diethyl fumarate; x represents the fractional content of group A, which ranges from 0.03 to less than 0.1 mol/mol of polymer of formula (I); y represents the fractional content of group B, which ranges from 0.50 to 0.97 mol/mol of polymer of formula (I); and z represents the fractional content of group C, which ranges from 0 to 0.47 mol/mol of polymer of formula (I), and formula (II) is represented by



wherein X, Y and Z each represents hydrogen, an alkyl group having from 1 to 6 carbon atoms, —COR, or —COOR<sub>1</sub>; Q represents



and R represents



where R<sub>1</sub> represents a substituted or an unsubstituted alkyl group having from 1 to 18 carbon atoms, an aryl group having from 6 to 18 carbon atoms, or an aralkyl group having from 7 to 12 carbon atoms; R<sub>2</sub> represents hydrogen, a halogen atom, an alkyl group having from 1 to 12 carbon atoms or an alkoxy group having from 1 to 6 carbon atoms; R<sub>3</sub> represents hydrogen, a substituted or an unsubstituted alkyl group having from 1 to 4 carbon atoms, a phenyl group or an aralkyl group having from 7 to 10 carbon atoms; R<sub>4</sub> represents the same groups as R<sub>3</sub> or an —R<sub>5</sub>—CONH)R<sub>5</sub>—COR<sub>7</sub> group, wherein R<sub>5</sub> represents a divalent aliphatic or an aromatic group (C<sub>1</sub>—C<sub>12</sub>), R<sub>7</sub> represents —OM, hydrogen, a substituted or an unsubstituted alkyl group (C<sub>1</sub>—C<sub>4</sub>), a phenyl group or an aralkyl group (C<sub>7</sub>—C<sub>10</sub>) and 1 is an integer of 0 to 6; M represents hydrogen or a cation; m is 0 or 1; and n is an integer of 1 to 4; and formula (III) is represented by

40

45

50

55

60

65



wherein D and E each represents hydrogen, a methyl group, a halogen atom, or —COOR<sub>6</sub>; G represents hydrogen, a methyl group, a halogen atom or —(CH<sub>2</sub>)<sub>k</sub>—COOR<sub>6</sub>; J represents hydrogen, an aryl group,



R<sub>6</sub> represents a substituted or an unsubstituted alkyl group having from 1 to 10 carbon atoms, an aryl group having from 6 to 12 carbon atoms, or an aralkyl group having from 7 to 12 carbon atoms; and k is 0 or 1.

20

12. A method as in claim 11, wherein said divalent group A is represented by the formula (II) wherein X, Y and Z each is hydrogen, a methyl group or —COR, and Q is —(CH<sub>2</sub>)<sub>m</sub>—.

13. A method as in claim 11, wherein said formula (II) represents acrylic acid, methacrylic acid, maleic acid, itaconic acid or acryloylaminoo acid.

14. A method as in claim 11, wherein said formula (II) represents acrylic acid or methacrylic acid.

15. A method as in claim 11, wherein said divalent group B is represented by the formula (III) wherein D and E each is hydrogen and G is a methyl group.

16. A method as in claim 11, wherein said formula (III) represents a methacrylic acid ester or a styrene.

17. A method as in claim 11, wherein said formula (II) represents acrylic acid or methacrylic acid, and said formula (III) represents a methacrylic acid ester or a styrene.

18. A method as in claim 17, wherein z in said formula (I) is zero.

19. A method as in claim 11, 12, 13, 14, 15, 16, 17, or 18, wherein said outermost layer is a surface protecting layer, and said polymer grains are coated in an amount of from 2 to 500 mg per square meter.

20. A method as in claim 11, 12, 13, 14, 15, 16, 17, or 18, wherein the average grain diameter of the polymeric grains is from 1 $\mu$  to 8 $\mu$ .

21. A method as in claim 11, wherein said squeezing means is a rubber lips, squeeze rollers or buff rollers.

\* \* \* \* \*